

**United States Patent** [19]  
**Wollenberg**

[11] **Patent Number:** **4,617,138**  
[45] **Date of Patent:** **Oct. 14, 1986**

[54] **MODIFIED SUCCINIMIDES (II)**

[75] **Inventor:** **Robert H. Wollenberg**, San Rafael, Calif.

[73] **Assignee:** **Chevron Research Company**, San Francisco, Calif.

[21] **Appl. No.:** **722,882**

[22] **Filed:** **Apr. 12, 1985**

[51] **Int. Cl.<sup>4</sup>** ..... **C10M 105/50; C10M 105/56**

[52] **U.S. Cl.** ..... **252/51.5 A**

[58] **Field of Search** ..... **252/51.5 A**

[56] **References Cited**

**U.S. PATENT DOCUMENTS**

3,400,075 9/1968 Grimm et al. ..... 252/51.5 A  
3,438,899 4/1969 Benoit, Jr. ..... 252/51.5 A  
3,630,902 12/1971 Coupland et al. ..... 252/51.5 A  
3,897,454 7/1975 Hankins et al. ..... 252/51.5 A  
4,482,464 11/1984 Karol et al. ..... 252/51.5 A

**FOREIGN PATENT DOCUMENTS**

1318874 5/1973 United Kingdom ..... 252/51.5 A

*Primary Examiner*—William R. Dixon, Jr.

*Assistant Examiner*—Margaret B. Medley

*Attorney, Agent, or Firm*—S. R. LaPaglia; R. C. Gaffney; G. F. Swiss

[57] **ABSTRACT**

Disclosed are polyamino alkenyl or alkyl succinimides which have been modified by treatment with a lactone to yield polyamino alkenyl or alkyl succinimides wherein one or more of the basic nitrogens of the polyamino moiety is substituted with a hydrocarbylcarbonylalkylene group. The additives so disclosed are useful as dispersants in lubricating oils, gasolines, marine crankcase oils and hydraulic oils.

**12 Claims, No Drawings**

## MODIFIED SUCCINIMIDES (II)

## BACKGROUND OF THE INVENTION

## 1. Field of the Invention

This invention relates to additives which are useful as dispersants and/or detergents in lubricating oils. In particular, this invention is directed toward polyamino alkenyl or alkyl succinimides which have been modified by treatment with a compound of the formula



wherein R is alkyl of 1 to 2 carbon atoms; R<sub>7</sub> is hydrocarbyl of from 1 to 30 carbon atoms; n is an integer of from 0 to 3; and p is an integer equal to 0 or 1. The modified alkenyl or alkyl succinimides of this invention have been found to possess dispersancy and/or detergency properties in lubricating oil. These modified succinimides are also useful as detergents and/or dispersants in fuels.

## 2. Prior Art

Alkenyl or alkyl succinimides have been previously modified with hydroxy alkylene acids selected from glycolic, lactic, 2-hydroxymethylpropionic and 2,2'-bis-hydroxymethylpropionic acids. The hydroxy alkylene acids react with either a primary or secondary amine to form a hydroxy alkylene amide. These modified succinimides are taught as additives for lubricating oils (see Karol, U.S. Pat. No. 4,482,464). However, there is no teaching in these patents, or apparently elsewhere, to modify alkenyl or alkyl succinimides with the lactones employed in this invention.

## SUMMARY OF THE INVENTION

It has now been found that polyamino alkenyl or alkyl succinimides may be modified by reaction with a lactone of the formula:



wherein R is alkyl of from 1 to 2 carbon atoms; R<sub>7</sub> is hydrocarbyl of from 1 to 30 carbon atoms; n is an integer of from 0 to 3; and p is an integer of from 0 to 1. The lactone reacts with the alkenyl or alkyl succinimide by adding a hydrocarbylcarbonylalkylene group to a primary or secondary amine with the concomitant elimination of CO<sub>2</sub>. Accordingly, the present invention relates to a polyamino alkenyl or alkyl succinimide wherein one or more of the basic nitrogens of the polyamino moiety is substituted with a hydrocarbylcarbonylalkylene group wherein said hydrocarbyl contains from 1 to 30 carbon atoms and alkylene is a three or four carbon alkylene group or a three or four carbon alkylene group substituted with from 1 to 3 alkyl groups of from 1 to 2 carbons each.

In general, the alkenyl or alkyl group of the succinimide is from 10 to 300 carbon atoms. While the modified succinimides of this invention possess good deter-

gancy properties even for alkenyl or alkyl groups of less than 20 carbon atoms, dispersancy is enhanced when the alkenyl or alkyl group is at least 20 carbon atoms. Accordingly, in a preferred embodiment, the alkenyl or alkyl group of the succinimide is at least 20 carbon atoms.

As noted above, the modified polyamino alkenyl or alkyl succinimides of this invention possess dispersancy and/or detergency properties when used in either lubricating oils or fuels. Thus, another aspect of this invention is a lubricating oil composition comprising a major amount of an oil of lubricating viscosity and an amount of a modified polyamino alkenyl or alkyl succinimide sufficient to provide dispersancy and/or detergency.

In another aspect of this invention is a fuel composition comprising a major portion of a hydrocarbon boiling in a gasoline or diesel range and an amount of a modified polyamino alkenyl or alkyl succinimide sufficient to provide dispersancy and/or detergency.

In still another aspect of the instant invention is a process for preparing polyamino alkenyl or alkyl succinimides wherein one or more of the basic nitrogens of the polyamino moiety is substituted with a hydrocarbylcarbonylalkylene group wherein said hydrocarbyl contains 1 to 30 carbon atoms; alkylene is a 3 or 4 carbon alkylene optionally substituted with from 1 to 3 alkyl groups of 1 to 2 carbons each; which comprises contacting at a temperature sufficient to cause reaction a lactone of Formula I with an alkenyl or alkyl succinimide.

## DETAILED DESCRIPTION OF THE INVENTION

The modified polyamino alkenyl or alkyl succinimides of this invention are prepared by reaction of a polyamino alkenyl or alkyl succinimide with a lactone of formula I above. The reaction is conducted at a temperature sufficient to cause reaction of the lactone with the polyamino alkenyl or alkyl succinimide. In particular, reaction temperatures of from about 0° C. to about 250° C. are preferred with temperatures of from about 100° C. to 200° C. being most preferred.

The reaction may be conducted neat—that is, both the polyamino alkenyl or alkyl succinimide and the lactone are combined in the proper ratio, either alone or in the presence of a catalyst, such as an acidic, basic or Lewis acid catalyst, and then stirred at the reaction temperature. Examples of suitable catalysts include, for instance, boron trifluoride, alkane sulfonic acid, alkali or alkaline carbonate.

Alternatively, the reaction may be conducted in a diluent. For example, the reactants may be combined in a solvent such as toluene, xylene, oil or the like, and then stirred at the reaction temperature. After reaction completion, volatile components may be stripped off. When a diluent is employed, it is preferably inert to the reactants and products formed and is generally used in an amount sufficient to insure efficient stirring.

Water, which can be present in the polyamino alkenyl or alkyl succinimide, may be removed from the reaction system either before or during the course of the reaction via azeotroping or distillation. After reaction completion, the system can be stripped at elevated temperatures (100° C. to 250° C.) and reduced pressures to remove any volatile components which may be present in the product.

Another embodiment of the above process is a continuous flow system in which the alkenyl or alkyl suc-

cinic anhydride and polyamine are added at the front end of the flow while the lactone is added further downstream in the system.

Mole charge of the lactone to the basic amine nitrogen of the polyamino alkenyl or alkyl succinimide employed in the process of this invention are generally in the range of from about 0.2:1 to about 1:1, although preferably from about 0.5:1 to about 1:1 and most preferably from about 0.7:1 to about 1:1.

As used herein, the term "molar charge" of lactone to the basic nitrogen of a polyamino alkenyl or alkyl-succinimide" means that the molar charge of lactone employed in the reaction is based upon the theoretical number of basic nitrogens contained in the succinimide. Thus, when 1 equivalent of triethylene tetraamine (TETA) is reacted with an equivalent of succinic anhydride, the resulting monosuccinimide will theoretically contain 3 basic nitrogens. Accordingly, a molar charge of 1 would require that a mole of lactone be added for each basic nitrogen or in this case 3 moles of lactone for each mole of monosuccinimide prepared from TETA.

The reaction is generally complete from within 0.5 to 10 hours.

#### A. POLYAMINO ALKENYL OR ALKYL SUCCINIMIDES

The polyamino alkenyl or alkyl succinimides that can be used to prepare the lubricating oil additives described herein are disclosed in numerous references and are well known in the art. Certain fundamental types of succinimides and related materials encompassed by the term of art "succinimide" are taught in U.S. Pat. Nos. 2,992,708; 3,018,291; 3,024,237; 3,100,673; 3,219,666; 3,172,892; and 3,272,746, the disclosures of which are hereby incorporated by reference. The term "succinimide" is understood in the art to include many of the amide, imide and amidine species which are also formed by this reaction. The predominant product however is succinimide and this term has been generally accepted as meaning the product of a reaction of an alkenyl substituted succinic acid or anhydride with a polyamine. As used herein, included within this term are the alkenyl or alkyl mono-, bis-succinimides and other higher analogs.

##### A(1) Succinic Anhydride

The preparation of the alkenyl-substituted succinic anhydride by reaction with a polyolefin and maleic anhydride has been described, e.g., U.S. Pat. Nos. 3,018,250 and 3,024,195. Such methods include the thermal reaction of the polyolefin with maleic anhydride and the reaction of a halogenated polyolefin, such as a chlorinated polyolefin, with maleic anhydride. Reduction of the alkenyl-substituted succinic anhydride yields the corresponding alkyl derivative. Alternatively, the alkenyl substituted succinic anhydride may be prepared as described in U.S. Pat. Nos. 4,388,471 and 4,450,281 which are totally incorporated herein by reference.

Polyolefin polymers for reaction with the maleic anhydride are polymers comprising a major amount of C<sub>2</sub> to C<sub>5</sub> mono-olefin, e.g., ethylene, propylene, butylene, isobutylene and pentene. The polymers can be homopolymers such as polyisobutylene as well as copolymers of 2 or more such olefins such as copolymers of: ethylene and propylene, butylene, and isobutylene, etc. Other copolymers include those in which a minor amount of the copolymer monomers, e.g., 1 to 20 mole percent is a C<sub>4</sub> to C<sub>8</sub> non-conjugated diolefin, e.g., a

copolymer of isobutylene and butadiene or a copolymer of ethylene, propylene and 1,4-hexadiene, etc.

The polyolefin polymer usually contains from about 10 to 300 carbon atoms, although preferably 10 to 200 carbon atoms and most preferably 20 to 100 carbon atoms.

A particularly preferred class of olefin polymers comprises the polybutenes, which are prepared by polymerization of one or more of 1-butene, 2-butene and isobutene. Especially desirable are polybutenes containing a substantial proportion of units derived from isobutene. The polybutene may contain minor amounts of butadiene which may or may not be incorporated in the polymer. Most often the isobutene units constitute 80%, preferably at least 90%, of the units in the polymer. These polybutenes are readily available commercial materials well known to those skilled in the art. Disclosures thereof will be found, for example, in U.S. Pat. Nos. 3,215,707; 3,231,587; 3,515,669; and 3,579,450, as well as U.S. Pat. No. 3,912,764. The above are incorporated by reference for their disclosures of the suitable polybutenes.

In addition to the reaction of a polyolefin with maleic anhydride, many other alkylating hydrocarbons may likewise be used with maleic anhydride to produce alkenyl succinic anhydride. Other suitable alkylating hydrocarbons include cyclic, linear, branched and internal or alpha olefins with molecular weights in the range 100-4,500 or more with molecular weights in the range of 200-2,000 being more preferred. For example, alpha olefins obtained from the thermal cracking of paraffin wax. Generally, these olefins range from 5-20 carbon atoms in length. Another source of alpha olefins is the ethylene growth process which gives even number carbon olefins. Another source of olefins is by the dimerization of alpha olefins over an appropriate catalyst such as the well known Ziegler catalyst. Internal olefins are easily obtained by the isomerization of alpha olefins over a suitable catalyst such as silica.

##### A(2) Polyamine

The polyamine employed to prepare the polyamino alkenyl or alkyl succinimides is preferably a polyamine having from 2 to about 12 amine nitrogen atoms and from 2 to about 40 carbon atoms. The polyamine is reacted with an alkenyl or alkyl succinic anhydride to produce the polyamino alkenyl or alkyl succinimide, employed in this invention. The polyamine is so selected so as to provide at least one basic amine per succinimide. Since the reaction of the polyamino alkenyl or alkyl succinimide with the lactones employed in this invention is believed to proceed through a secondary or primary amine, at least one of the basic amine atoms of the polyamino alkenyl or alkyl succinimide must either be a primary amine or a secondary amine. Accordingly, in those instances in which the succinimide contains only one basic amine, that amine must either be a primary amine or a secondary amine. The polyamine preferably has a carbon-to-nitrogen ratio of from about 1:1 to about 10:1.

The polyamine portion of the polyamino alkenyl or alkyl succinimide may be substituted with substituents selected from (A) hydrogen, (B) hydrocarbyl groups of from 1 to about 10 carbon atoms, (C) acyl groups of from 2 to about 10 carbon atoms, and (D) monoketo, monohydroxy, mononitro, monocynano, lower alkyl and lower alkoxy derivatives of (B) and (C)/ "Lower", as used in terms like lower alkyl or lower alkoxy, means a

group containing from 1 to about 6 carbon atoms. At least one of the substituents on one of the amines of the polyamine is hydrogen, e.g., at least one of the basic nitrogen atoms of the polyamine is a primary or secondary amino nitrogen atom.

Hydrocarbyl, as used in describing the polyamine substituents and R<sub>7</sub> group, denotes an organic radical composed of carbon and hydrogen which may be aliphatic, alicyclic, aromatic or combinations thereof, e.g., aralkyl. Preferably, the hydrocarbyl group will be relatively free of aliphatic unsaturation, i.e., ethylenic and acetylenic, particularly acetylenic unsaturation. The substituted polyamines of the present invention are generally, but not necessarily, N-substituted polyamines. Exemplary hydrocarbyl groups and substituted hydrocarbyl groups include alkyls such as methyl, ethyl, propyl, butyl, isobutyl, pentyl, hexyl, octyl, etc., alkenyls such as propenyl, isobut enyl, hexenyl, octenyl, etc., hydroxyalkyls, such as 2-hydroxyethyl, 3-hydroxypropyl, hydroxyisopropyl, 4-hydroxybutyl, etc., ketoalkyls, such as 2-ketopropyl, 6-ketoctyl, etc., alkoxy and lower alkenoxy alkyls, such as ethoxyethyl, ethoxypropyl, propoxyethyl, propoxypropyl, 2-(2-ethoxyethoxyethyl, 2-(2-(2-ethoxyethoxy)ethoxyethyl, 3,6,9,12-tetraoxatetradecyl, 2-(2-ethoxyethoxy)hexyl, etc. The acyl groups of the aforementioned (C) substituents are such as propionyl, acetyl, etc. The more preferred substituents are hydrogen, C<sub>1</sub>-C<sub>6</sub> alkyls and C<sub>1</sub>-C<sub>6</sub> hydroxylalkyls.

In a substituted polyamine the substituents are found at any atom capable of receiving them. The substituted atoms, e.g., substituted nitrogen atoms, are generally geometrically inequivalent, and consequently the substituted amines finding use in the present invention can be mixtures of mono- and polysubstituted polyamines with substituent groups situated at equivalent and/or inequivalent atoms.

The more preferred polyamine finding use within the scope of the present invention is a polyalkylene polyamine, including alkylene diamine, and including substituted polyamines, e.g., alkyl and hydroxyalkyl-substituted polyalkylene polyamine. Preferably, the alkylene group contains from 2 to 6 carbon atoms, there being preferably from 2 to 3 carbon atoms between the nitrogen atoms. Such groups are exemplified by ethylene, 1,2-propylene, 2,2-dimethyl-propylene, trimethylene, 1,3,2-hydroxypropylene, etc. Examples of such polyamines include ethylene diamine, diethylene triamine, di(trimethylene)triamine, dipropylene triamine, triethylene tetramine, tripropylene tetramine, tetraethylene pentamine, and pentaethylene hexamine. Such amines encompass isomers such as branched-chain polyamines and the previously mentioned substituted polyamines, including hydroxy- and hydrocarbyl-substituted polyamines. Among the polyalkylene polyamines, those containing 2-12 amine nitrogen atoms and 2-24 carbon atoms are especially preferred, and the C<sub>2</sub>-C<sub>5</sub> alkylene polyamines are most preferred, in particular, the lower polyalkylene polyamines, e.g., ethylene diamine, dipropylene triamine, etc.

The polyamine component also may contain heterocyclic polyamines, heterocyclic substituted amines and substituted heterocyclic compounds, wherein the heterocycle comprises one or more 5-6 membered rings containing oxygen and/or nitrogen. Such heterocycles may be saturated or unsaturated and substituted with groups selected from the aforementioned (A), (B), (C) and (D). The heterocycles are exemplified by piper-

zines, such as 2-methylpiperazine, N-(2-hydroxyethyl)piperazine, 1,2-bis-(N-piperazinyl)ethane, and N,N'-bis(N-piperazinyl)piperazine, 2-methylimidazoline, 3-aminopiperidine, 2-aminopyridine, 2-(3-aminoethyl)-3-pyrroline, 3-aminopyrrolidine, N-(3-aminopropyl)morpholine, etc. Among the heterocyclic compounds, the piperazines are preferred.

Typical polyamines that can be used to form the compounds of this invention include the following: 10 ethylene diamine, 1,2-propylene diamine, 1,3-propylene diamine, diethylene triamine, triethylene tetramine, hexamethylene diamine, tetraethylene pentamine, methylaminopropylene diamine, N-(betaaminoethyl)piperazine, N-(betaaminoethyl)piperidine, N-(beta-aminoethyl)morpholine, N,N'-di(betaaminoethyl)piperazine, 15 N,N'-di(betaaminoethyl)imidazolidone-2, N-(beta-cyanoethyl)ethane-1,2-diamine, 1,3,6,9-tetraaminooctadecane, 1,3,6-triamino-*b*-9-oxadecane, N-(beta-aminoethyl)diethanolamine, N'-acetyl-N'-methyl-N-(beta-aminoethyl)-ethanol, 20 2-diamen, N-methyl-1,2-propanediamine, N-(beta-nitroethyl)-1,3-propane diamine, 5-(beta-aminoethyl)-1,3,5-dioxazine, 2-(2-aminoethylamino)-ethanol, 2-[2-(2-aminoethylamino)-ethylamino]-ethanol.

Another group of suitable polyamines are the propyleneamines, (bisaminopropylethylenediamines). Propyleneamines are prepared by the reaction of acrylonitrile with an ethyleneamine, for example, an ethyleneamine having the formula 30 H<sub>2</sub>N(CH<sub>2</sub>CH<sub>2</sub>NH)<sub>Z</sub>H wherein Z is an integer from 1 to 5, followed by hydrogenation of the resultant intermediate. Thus, the product prepared from ethylene diamine and acrylonitrile would be H<sub>2</sub>N(CH<sub>2</sub>)<sub>3</sub>NH(CH<sub>2</sub>)<sub>2</sub>NH(CH<sub>2</sub>)<sub>3</sub>NH<sub>2</sub>.

In many instances the polyamine used as a reactant in the production of succinimides of the present invention is not a single compound but a mixture in which one or several compounds predominate with the average composition indicated. For example, tetraethylene pentamine prepared by the polymerization of aziridine or the reaction of dichloroethylene and ammonia will have both lower and higher amine members, e.g., triethylene tetramine, substituted piperazines and pentaethylene hexamine, but the composition will be largely tetraethylene pentamine and the empirical formula of the total amine composition will closely approximate that of tetraethylene pentamine. Finally, in preparing the succinimide for use in this invention, where the various nitrogen atoms of the polyamine are not geometrically equivalent, several substitutional isomers are possible and are encompassed within the final product. Methods of preparation of polyamines and their reactions are detailed in Sidgewick's "The Organic Chemistry of Nitrogen", Clarendon Press, Oxford, 1966; Noller's "Chemistry of Organic Compounds", Saunders, Philadelphia, 2nd Ed., 1957; and Kirk-Othmer's "Encyclopedia of Chemical Technology", 2nd Ed., especially Volumes 2, pp. 99-116.

The reaction of a polyamine with an alkenyl or alkyl 60 succinic anhydride to produce the alkenyl or alkyl succinimides is well known in the art and is disclosed in U.S. Pat. Nos. 2,992,708; 3,018,291; 3,024,237; 3,100,673; 3,219,666; 3,172,892 and 3,272,746. The above are incorporated herein by reference for their disclosures of preparing alkenyl or alkyl succinimides.

As noted above, the term "polyamino alkenyl or alkyl succinimide" refers to both polyamino alkenyl or alkyl mono- and bis-succinimides and to the higher analogs of

polyamino alkenyl or alkyl poly succinimides. Preparation of the bis- and higher analogs may be accomplished by controlling the molar ratio of the reagents. For example, a product comprising predominantly mono- or bis-succinimide can be prepared by controlling the molar ratios of the polyamine and succinic anhydride. Thus, if one mole of polyamine is reacted with one mole of an alkenyl or alkyl substituted succinic anhydride, a predominantly mono-succinimide product will be prepared. If two moles of an alkenyl substituted succinic anhydride are reacted per mole of polyamine, a bis-succinimide is prepared. Higher analogs may likewise be prepared.

A particularly preferred class of polyamino alkenyl or alkyl succinimides employed in the process of the instant invention may be represented by Formula II:



wherein R<sub>1</sub> is alkenyl or alkyl of from 10 to 300 carbon atoms; R<sub>2</sub> is alkylene of 2 to 10 carbon atoms; R<sub>3</sub> is hydrogen or lower alkyl of from 1 to 6 carbon atoms; a is an integer from 0 to 10; and W is —NH<sub>2</sub> or represents a group of Formula III:



wherein R<sub>1</sub> is alkenyl or alkyl of from 10 to 300 carbon atoms; with the proviso that when W is the group of Formula III above, then a is not zero and at least one of R<sub>3</sub> is hydrogen.

As indicated above, the polyamine employed in preparing the succinimide is often a mixture of different compounds having an average composition indicated as in Formula IV below:



wherein R<sub>2</sub>, R<sub>3</sub> and a are as defined above. Accordingly, in Formula IV each value of R<sub>2</sub> and a may be the same or different from other values of R<sub>2</sub> and a. Moreover, cyclic heterocycles, such as piperazine, may be included to some extent in the alkylene diamines, IV.

Preferably, R<sub>2</sub> is alkylene of 2 to 6 carbon atoms and most preferably is either ethylene or propylene.

Preferably, R<sub>3</sub> is hydrogen while a is preferably an integer from 1 to 6.

In Formula II, the polyamino alkenyl or alkyl succinimides may be conveniently viewed as being composed of three moieties that is the alkenyl or alkyl moiety, R<sub>1</sub>, the succinimide moiety represented by the formula:



10 and the polyamino moiety represented by the group



## B. LACTONES

The lactones employed in this invention may be represented by the formula:



wherein R is alkyl of 1 to 2 carbon atoms; R<sub>7</sub> is hydrocarbyl of from 1 to 30 carbons atoms; n is an integer of from 0 to 3; and p is an integer of from 0 to 1. Preferably, R<sub>7</sub> is hydrocarbyl of from 1 to 10 carbon atoms; preferably n is equal to either 0 or 1 while R is preferably methyl. Most preferably, n is zero.

35 The 2-hydrocarbylcarbonyl substituted lactones of Formula I above are conveniently prepared by treating the lactone, V, with a base, b, and then adding as ester, VI, as shown in reaction (1) below



40 wherein R, R<sub>7</sub>, n and p are as defined above and R<sub>8</sub> is alkyl of 1 or 2 carbon atoms and b is an organic or inorganic base. The reaction is conducted by first combining the base, b, with the lactone, V, preferably in an inert diluent such as toluene, chloroform, methylene chloride, and the like. The ester, VI, is then added to the system. Suitable bases for use in this reaction include organic bases such as sodium methoxide, potassium methoxide, sodium ethoxide and the like; and inorganic bases such as sodium hydroxide, potassium hydroxide and the like. Generally the reaction is at room temperature to the reflux temperature of the diluent employed. The reaction is generally complete within from  $\frac{1}{2}$  to 24 hours. Afterwards the product, I, may be isolated by conventional techniques such as chromatography, filtration, etc., or may be used as is the reaction with a polyamino alkenyl or alkyl succinimide.

55 The lactones of Formula V above are either commercially available such as gamma butyrolactone and valerolactone or may be prepared by art recognized

procedures such as those disclosed in U.S. Pat. No. 4,309,352 and by Christian et al., "Journal American Chemical Society", 69, 1961-1963 (1947).

Lactones, V, which may be employed in reaction (1) include, for instance, gamma butyrolactone, gamma valerolactone (tetrahydro-5-methyl-2-furanone), delta valerolactone, tetrahydro-5,5-dimethyl-2-furanone, 6-methyl delta valerolactone, 6-ethyl delta valerolactone, and the like.

### C. MODIFIED SUCCINIMIDE COMPLEXES

The lactones of this invention react with primary and secondary amines of a polyamino alkenyl or alkyl succinimide by adding a hydrocarbylcarbonylalkylene group to the amine. This is illustrated in reaction (2) below which employs 2-hydrocarbylcabonyl gamma butyrolactone for illustrative purposes. It is understood that other lactones react similarly.



olefins such as 1-decene trimer. Likewise, alkyl benzenes of proper viscosity such as didodecyl benzene, can be used. Useful synthetic esters include the esters of both monocarboxylic acid and polycarboxylic acids as well as monohydroxy alkanols and polyols. Typical examples are didodecyl adipate, pentaerythritol tetracaproate, di-2-ethylhexyl adipate, dilaurylsebacate and the like. Complex esters prepared from mixtures of mono and dicarboxylic acid and mono and dihydroxy alkanols can also be used.

Blends of hydrocarbon oils with synthetic oils are also useful. For example, blends of 10 to 25 weight percent hydrogenated 1-decene trimer with 75 to 90 weight percent 150 SUS (100° F.) mineral oil gives an excellent lubricating oil base.

Additive concentrates are also included within the scope of this invention. The concentrates of this invention usually include from about 90 to 10 weight percent of an oil of lubricating viscosity and from about 10 to 90 weight percent of the complex additive of this invention. Typically, the concentrates contain sufficient diluent to make them easy to handle during shipping and storage. Suitable diluents for the concentrates include any inert diluent, preferably an oil of lubricating viscosity, so that the concentrate may be readily mixed with lubricating oils to prepare lubricating oil compositions. Suitable lubricating oils which can be used as diluents typically have viscosities in the range from about 35 to about 500 Saybolt Universal Seconds (SUS) at 100° F. (38° C.), although an oil of lubricating viscosity may be used.

Other additives which may be present in the formulation include rust inhibitors, foam inhibitors, corrosion inhibitors, metal deactivators, pour point depressants, antioxidants, and a variety of other well-known additives.

It is also contemplated the modified succinimides of this invention may be employed as dispersants and detergents in hydraulic fluids, marine crankcase lubricants and the like. When so employed, the modified succinimide is added at from about 0.1 to 10 percent by weight to the oil. Preferably, at from 0.5 to 5 weight percent.

When used in fuels, the proper concentration of the additive necessary in order to achieve the desired detergency is dependent upon a variety of factors including the type of fuel used, the presence of other detergents or dispersants or other additives, etc. Generally, however, and in the preferred embodiment, the range of concentration of the additive in the base fuel is 10 to 10,000 weight parts per million, preferably from 30 to 2,000 weight parts per million, and most preferably from 30 to 700 parts per million of the modified succinimide per part of base fuel. If other detergents are present, a lesser amount of the modified succinimide may be used.

The modified succinimide additives of this invention may be formulated as a fuel concentrate, using an inert stable oleophilic organic solvent boiling in the range of about 150° to 400° F. Preferably, an aliphatic or an aromatic hydrocarbon solvent is used, such as benzene, toluene, xylene or higher-boiling aromatics or aromatic thinners. Aliphatic alcohols of about 3 to 8 carbon atoms, such as isopropanol, isobutylcarbinol, n-butanol and the like, in combination with hydrocarbon solvents are also suitable for use with the fuel additive. In the fuel concentrate, the amount of the additive will be ordinarily at least 10 percent by weight and generally not exceed 70 percent by weight and preferably from 10 to 25 weight percent.

The following examples are offered to specifically illustrate this invention. These examples and illustrations are not to be construed in any way as limiting the scope of this invention.

### EXAMPLE

To a 500 ml reaction flask was charged 253.4 g of a succinimide dispersant composition [prepared from 1 mole of polyisobutylsuccinic anhydride, where the polyisobutyl group has a number average molecular weight of 950, and triethylenetetraamine and which consists of about 50% lubricating oil diluent and having alkalinity value (AV) of 47 mg KOH/g]. To this succinimide was added 38.4 g of 2-acetylbutyrolactone. The mixture was heated under nitrogen to 150±5° C. for 10 hrs. Recovered product containing 2.04%N and having an AV=33.1 mg KOH/g.

What is claimed is:

1. A polyamino alkenyl or alkyl succinimide wherein one or more of the basic nitrogens of the polyamino moiety is substituted with a hydrocarbylcarbonylalkylene wherein said hydrocarbylcarbonyl group contains 1 to 30 carbon atoms; said alkylene is a three or four carbon alkylene group or a three of four carbon alkylene group substituted with from 1 to 3 alkyl groups of from 1 to 2 carbons each.
2. The polyamino alkenyl or alkyl succinimide of claim 1 wherein said alkylene is a three or four carbon alkylene group.
3. The polyamino alkenyl or alkyl succinimide of claim 2 wherein said alkylene is propylene.
4. The polyamino alkenyl or alkyl succinimide of claim 2 wherein said alkylene is butylene.
5. The polyamino alkenyl or alkyl succinimide of claim 1 wherein said alkylene is a three or four carbon alkylene group substituted with from 1 to 3 alkyl groups of from 1 to 2 carbons each.
6. The polyamino alkenyl or alkyl succinimide of claim 1 wherein said hydrocarbylcarbonylalkylene is methylcarbonylpropylene (i.e.,



7. A compound of the formula:



wherein R<sub>1</sub> is alkenyl or alkyl of from 10 to 300 carbon atoms; R<sub>2</sub> is alkylene of 2 to 10 carbon atoms; R<sub>6</sub> is hydrogen, lower alkyl of from 1 to 6 carbon atoms, and hydrocarbylcarbonylalkylene wherein said hydrocarbyl contains from 1 to 30 carbon atoms; said alkylene is a three or four carbon alkylene group or a three or four carbon alkylene group substituted with from 1 to 3 alkyl groups of from 1 to 2 carbon atoms each; a is an integer of from 1 to 6; and T is  $-\text{N}(\text{R}_6)_2$ ,  $-\text{NHR}_6$  and



wherein R<sub>6</sub> is as defined above and R<sub>1</sub> is alkenyl or alkyl of from 10 to 300 carbon atoms, with the proviso that the compound contains at least one R<sub>6</sub> which is hydrocarbylcarbonylalkylene.

8. A lubricating oil composition comprising an oil of lubricating viscosity and an amount effective to provide dispersancy of a compound as defined in claim 7.

9. A lubricating oil concentrate comprising from about 90 to 10 weight percent of an oil of lubricating viscosity and from about 10 to 90 weight percent of a compound as defined in claim 7.

10. A compound as defined in claim 7 wherein R<sub>1</sub> is alkenyl or alkyl of from 20 to 100 carbon atoms.

10 11. A compound as defined in claim 10 wherein R<sub>2</sub> is alkylene of from 2 to 6 carbon atoms.

12. A compound as defined in claim 11 wherein the hydrocarbylcarbonylalkylene group is methylcarbonyl propylene.

\* \* \* \* \*

15

20

25

30

35

40

45

50

55

60

65